

Sept. 6, 1955

S. A. SIMON ET AL

2,717,193

BLEACHING PROCESS FOR COTTON OF LOW GRADE FOR COLOR

Filed Nov. 19, 1952

2 Sheets-Sheet 1



T1Q1.



T1Q2.

INVENTORS:

SIMON A. SIMON

HARVEY C. RUHE.

BY

Leroy F. Kelley

ATTORNEY

Sept. 6, 1955

S. A. SIMON ET AL

2,717,193

BLEACHING PROCESS FOR COTTON OF LOW GRADE FOR COLOR

Filed Nov. 19 1952

2 Sheets-Sheet 2



INVENTORS:  
SIMON A. SIMON  
HARVEY C. RUHF

BY *LeRoy T. Holley*  
ATTORNEY

% REFLECTANCE OF BLEACHED COTTON

1

2,717,193

## BLEACHING PROCESS FOR COTTON OF LOW GRADE FOR COLOR

Simon A. Simon, Longmeadow, and Harvey Clayton Ruhf, Springfield, Mass., assignors to Chicopee Manufacturing Corporation, a corporation of Massachusetts

Application November 19, 1952, Serial No. 321,378

14 Claims. (Cl. 8—111)

This invention relates to the bleaching of cotton, either woven or nonwoven, and more particularly relates to an improved process for the bleaching of cotton of low grade for color, although the invention has application to the bleaching of higher grades of cotton.

It has long been recognized in the textile industry that there is a problem associated with the bleaching of cotton of low grade for color; also variously referred to as definitely shaded cotton, blue cotton, discolored cotton, light gray cotton, gray cotton, dull cotton, off-cotton and off-shades of cotton; not encountered in the bleaching of the better grades of cotton which are called white or unshaded cotton. The desire has been repeatedly expressed in textile publications for a solution to the problem of bleaching cottons of low grade for color because of the many difficulties the use of such cottons presents. If discolored cottons having fibers that are but slightly off-shade are blended with higher grade cottons, woven into piece goods and bleached, the departure from white is so marked that no amount of bluing or tinting will change the apparent effect and any attempt made to hide the shading will result in a saddening of the natural brilliancy of the cotton. It is customary practice in the textile industry to avoid carefully the blending of discolored cottons with the whiter shades because the bleacher cannot whiten the blended cottons with any degree of economy and resultant strength of the fibers. Although the factors involved and responsible for the discoloration of cotton are known, it is recognized in the textile industry that no practical method of bleaching discolored cotton to the degree of whiteness associated with the bleaching of white cotton has been suggested or is known, even though a great amount of work has been done to develop a method for the satisfactory bleaching of such cotton.

A substantial amount of cotton is discolored and classed as dull or gray because the fibers have been subjected to the action of microorganisms having the ability to grow and multiply on the surface of fibers as well as to penetrate the fibers and multiply in the lumina. Many of the microorganisms are dark in color and their presence as discolored matter on the surface and in the lumina gives the fibers a dull or grayed appearance.

The cotton fiber shown in cross-section and magnification in Figure 1 is a typical fiber consisting of a characteristic flattened, twisted, irregular tube of cellulose 10, and a wall 12 surrounding a hollow space 14 called a lumen and shows microorganisms 16 growing on the outside of the wall of the fiber. Figure 1 also shows punctures 18 in the fiber wall and organisms 20 growing in the lumen of the fiber. Fibers in which there is growth of microorganisms in the lumina are duller and of lower grade for color and are least responsive to bleaching by conventional methods. Fibers in which the microorganisms have penetrated the cell wall and are present in the lumina do not respond satisfactorily to conventional methods of bleaching and do not provide bleached material having a degree of whiteness suitable for use in the manufacture of white cotton and white goods. Discolored cotton of this type

2

may be bleached to a satisfactory whiteness by subjecting it to a series of conventional bleaching cycles, but this results in a degradation of the cellulose molecules making up the fibers to such an extent that the cotton cannot be satisfactorily used in conventional textile processes.

Fabrics woven from this type of discolored cotton and subsequently bleached by repeated conventional bleaching operations do not have satisfactory laundering and wearing properties. Repeated bleaching of cotton results in damage to the fibers and markedly increases fiber fragility. Cotton having markedly increased fiber fragility is not acceptable for surgical uses because of the excessive amount of fly and fiber dust associated therewith.

It is an object of this invention to provide a process for the bleaching of cotton in general and cotton of low grade for color in particular, either in the form of fibers or fabric, to a satisfactory degree of whiteness without serious damage to the fibers and increase in fiber fragility.

It is another object of this invention to provide a process for the bleaching of discolored cotton, having discolored matter within the lumina of the fibers due to the action of microorganisms, to a satisfactory whiteness without serious damage to the fibers.

It is another and further object of this invention to provide a process by which cotton of low grade for color having a percent reflectance approximately within the range of from 64 Rd to 72 Rd is bleached in a single bleaching operation in batch or continuous method to a percent reflectance of not substantially less than 88.5 Rd.

The objects of this invention are accomplished by a bleaching process in which cotton fibers or cotton textiles remain in a substantially inactive bleaching bath containing a per compound as a bleaching agent, at a temperature of the bleaching bath below the temperature at which the

bleaching agent is activated and rapidly decomposed, for a latent period of time such that the bleaching agent is able to penetrate into the lumina of the fibers which contain discolored matter in the lumina. During the latent period, decomposition of the bleaching agent proceeds at a slow rate but a substantial amount remains undecomposed.

At the end of the latent period, the bleaching solution is activated and bleaching of the cotton continues until the discolored matter responsible for discoloring the fibers is bleached and the bleaching agent is exhausted.

In the drawings:

Figure 1 is a greatly magnified perspective in cross-section of a cotton fiber discolored by the action of microorganisms;

Figure 2 is a graph in which the percent reflectance of bleached cotton in Rd units is plotted against the percent of the hydrogen peroxide in the bleaching bath which is decomposed during the latent period and the curves in this graph show the relation between the time and temperature of the latent period to the percent reflectance in Rd units of bleached cotton as well as their relationship to the amount of bleaching agent decomposed during the latent period;

Figure 3 is a graph in which the percent reflectance of bleached cotton in Rd units is plotted against the time of the latent period and shows the relationship between the temperature of the bleaching solution during the latent period, the duration of the latent period and the percent reflectance of the bleached cotton.

The period of time during which the material to be bleached is kept in an inactive bleaching solution containing a per compound is at least about one and one-quarter hours but may be as long as twenty-four hours. If the time is substantially less than one and one-quarter hours, cotton fibers or woven materials, made from discolored fibers, and particularly made from fibers in which discolored material is present in the lumina of the fibers,

will not be bleached to a satisfactory whiteness. The time of the latent period may be considerably longer than one and one-quarter hours and even as long as twenty-four hours without any deleterious effect upon the fibers. The required time of the latent period is the shortest at a temperature of the bleaching bath of 50° C.; however, if the temperature of the bleaching bath is 15° C. or lower, the time of the steeping period must be at least about one and one-half hours. The time of the steeping period must also be at least about one and one-half hours if the temperature of the steeping bath is 55° C.

Bleaching agents satisfactory for use in the practice of this invention are generally referred to in the bleaching art as per compounds, and are compounds capable of releasing oxygen on activation. Aqueous solutions of hydrogen peroxide and sodium peroxide or per compounds which behave in solution as peroxides, such as sodium perborate and other inorganic perborate salts, are suitable for use in the bleaching process of this invention. Per compounds, when used as bleaching agents, may be conveniently maintained in a latent state, in which there is a minimum amount of decomposition and consequent exhaustion of their bleaching ability by the evolution of oxygen, by the presence in the bleaching solution of a substance such as sodium silicate which lends stability to the bleaching solution and is known as an "assistant." A bleaching solution, which has been maintained in an inactive state in the presence of assistants, may be activated by raising the temperature to a critical degree, by the addition of activators such as sodium carbonate and sodium hydroxide, or by raising the pH to about 12 or higher. The critical temperature and pH of such a bleaching solution varies with the per compound used and with the amount and kind of assistants present in the solution.

The whiteness of cotton in fiber or textile form is conventionally measured by means of an instrument known as the Hunter Color and Color Difference Meter, which measures diffused reflectance. Measurements of whiteness made by this method are called percent reflectance and are expressed in Rd units.

Chemical degradation of cotton is determined according to A. S. T. M. designation D539-40T. This method measures the fluidity of solutions of cotton and the measurements are expressed in rhes.

Reflectance, as measured according to the Hunter Color and Color Difference Meter, is uniform for cotton fibers, but varies with the number of threads per inch when reflectance measurements are made on cotton fabrics. A fabric having a lesser number of threads per inch will be lower in measured percent reflectance than a fabric having a greater number of threads per inch.

Unbleached or raw cotton is considered to be white or normal if it has a percent reflectance of 72 Rd or above. Cottons classed as dull have a percent reflectance of 64 Rd to 72 Rd. Cottons classed as gray have a percent reflectance of less than 64 Rd. A fabric is considered to have unsatisfactory laundering and wearing properties if the fibers have a fluidity of greater than 10 rhes. Cotton fibers having a percent reflectance of 88.5 Rd and above are referred to as "white" and cotton of this degree of whiteness is used by the medical and dental professions and in the home as such or in various forms such as pads, rolls and balls.

Cotton fibers can be prepared for bleaching according to the process of our invention by any of a variety of preliminary steps commonly practiced in preparing cotton fibers for conventional bleaching operations. A typical series of preparatory steps includes wet-out and desizing, washing, souring, washing, scouring and washing.

The following examples are given to illustrate the various modifications of the invention and to demonstrate the limits of the invention, but it is to be understood that they are presented only by way of illustration and that the invention is not to be restricted or limited thereby.

#### Example I

Ten-gram portions of kier-boiled cotton having a fluidity of 4 rhes and a percent reflectance in the raw state of 68 Rd were each immersed in 100 cc. of an aqueous bleaching solution containing 0.28 g. of hydrogen peroxide, 0.10 g. of sodium carbonate, and 0.10 g. of sodium silicate. Eight series of beakers, with eight beakers in a series, containing a cotton portion and bleaching solution were maintained each at a separate temperature for a latent period varying in length. The temperatures were 5° C., 15° C., 25° C., 40° C., 45° C., 50° C., 55° C., and 60° C. At each individual temperature the bleaching solution was immediately raised to a temperature of about 85° C. after fifteen minutes, thirty minutes, one and one-quarter, one and one-half, two, two and one-half, three, and twenty-four hours' immersion of the cotton in the bleaching solution. In all instances, after elevation of the temperature to 85° C., the solutions were held at that temperature until the bleaching agent was exhausted which required about two hours. The cotton samples were then removed from the bleaching solution and washed until clean and dried. The percent reflectance of each dried cotton sample was measured and the percent decomposition of the hydrogen peroxide during the steeping period was determined. Fluidities of all samples of bleached cotton were determined and were found to be between 4.5 and 5.5 rhes.

The results of the determination of the percent of the hydrogen peroxide in the bleaching bath decomposed at the eight different temperatures at which the cotton samples were immersed in the bleaching solution during latent periods of one, one and one-quarter, one and one-half, and two hours are given in the graph of Figure 2 as points on the curves. The results of determinations of percent reflectance in Rd units for cotton samples immersed in an inactive bleaching solution for all durations of the latent periods and at temperatures of 15° C., 25° C., 40° C., 45° C., 50° C., 55° C., and 60° C. are given in the graph of Figure 2 as points on the curves.

Figure 3 in particular shows in graphic form the relationship between the time of the latent period and the temperature of the bleaching solution during the latent period and the effect of these two conditions on the percent reflectance of the bleached cotton. It is apparent from an examination of Figure 3 that to obtain bleached cotton with a percent reflectance of 88.5 Rd, it is necessary that the material to be bleached remain in the steeping bath in an inactivated state for at least about one and one-quarter hours and that the time may only be this short if the temperature of the bleaching solution is 50° C. The results graphically shown in Figure 3 also show that if the temperature of the bleaching solution is below 50° C., the steeping time may be as short as one and one-half hours and that bleaching to a percent reflectance of 88.5 Rd is not accomplished when the temperature of the bleaching solution is substantially greater than about 55° C. It is preferred that the temperature of the bleaching solution be not substantially below 15° C. during the latent period, although discolored cotton may be bleached to a percent reflectance of 88.5 Rd at a temperature of the bleaching solution substantially below 15° C. when the time of the latent period is at least about one and one-half hours.

The graph of Figure 2 shows the relationship between the percent of the per compound, in this case hydrogen peroxide, which is decomposed during the latent period and the conditions of time and temperature to which the material to be bleached is subjected in the bleaching solution during the latent period and the effect of these conditions on the percent reflectance of the bleached cotton. The results presented graphically in Figure 2 show that if more than about 26 percent of the hydrogen peroxide is decomposed during a latent period of two hours, the cotton is not bleached to a percent reflectance of 88.5 Rd.

## Example II

Ten gram portions of kier-boiled cotton having a fluidity of 4 rhes and a percent reflectance in the raw state of 68 Rd were each immersed in 100 cc. of an aqueous bleaching solution containing 0.8 g. of sodium perborate, 0.1 g. sodium carbonate and 0.1 g. sodium silicate. Two beakers containing the cotton and bleaching solution were maintained at 25° C., one for one hour and the other for two hours, and then immediately raised to a temperature of about 85° C., at which temperature the bleaching agent was activated and active bleaching occurred. The temperature was held at 85° C. until the bleaching agent was exhausted. The cotton samples were removed from the exhausted bleaching solution, washed until clean and dried.

An additional two beakers containing the cotton and bleaching solution were maintained at a temperature of 50° C., one for a latent period of one hour, and the other two hours. After the latent period, the bleaching agent was activated by elevation of the temperature of the bleaching solution to 85° C. and bleaching of the cotton samples was finished as above.

The percent reflectance of each dried cotton sample was measured. Fluidities of all samples of bleached cotton were determined and were all found to be below 5 rhes. The results of this experiment are given in the table below in which percent reflectance is expressed in Rd units:

| Time           | Temperature,<br>° C. | Percent<br>Reflectance |
|----------------|----------------------|------------------------|
| One hour.....  | 25                   | 87.0                   |
| Two hours..... | 25                   | 89.5                   |
| One hour.....  | 50                   | 87.5                   |
| Two hours..... | 50                   | 90.0                   |

## Example III

A ten-gram portion of kier-boiled cotton having a fluidity of 3 rhes and a percent reflectance in the raw state of 68 Rd was bleached according to the bleaching procedure of Example I. The time of the latent period was two hours and the temperature of the bleaching solution during the latent period was 25° C. After the latent period, the temperature was immediately raised to 85° C. and held at that temperature until the bleaching agent was exhausted, which required about two hours. The cotton sample was then removed from the bleaching solution and washed until clean and dried. The fluidity of the bleached cotton sample was 4.6 rhes. The same sample of cotton was again subjected to bleaching according to the same conditions as in the first bleaching. The twice bleached cotton had a fluidity of 8 rhes. After a third and fourth bleaching under the same conditions, the fluidity of the cotton samples was 12 and 18 rhes, respectively.

## Example IV

Two ten-gram portions of a 28 x 24 fabric having a percent reflectance of 66.4 Rd were immersed in a bleaching bath having the same composition as that of Example I. The temperature of the bleaching solution in which one portion of fabric was immersed was held at 20° C. for a latent period of two hours and then rapidly elevated to 85° C. and maintained at that temperature for two hours. The bleaching agent was exhausted after two hours at 85° C. and the fabric was removed from the bleaching solution, washed and dried. The bleached fabric had a percent reflectance of 89.0 Rd and a fluidity of 4.5 rhes. The temperature of the bleaching solution in which the other portion of fabric was immersed was rapidly brought up to 85° C., immediately after immersion of the fabric in the bleaching solution. The temperature of the bleaching solution was maintained at 85° C. for two hours at which time the bleaching agent was exhausted. The fabric was removed from the bleaching

solution, washed, and dried, and had a percent reflectance of 80.0 Rd and a fluidity of 4.7 rhes.

A 28 x 24 cotton fabric is not considered white enough for surgical and household uses unless it has a percent reflectance of at least 83 Rd.

The results of the experiments show that cotton fibers having a percent reflectance in the raw state as low as 68 Rd may be satisfactorily bleached by a single bleaching operation in which no additional bleaching agent is added to the bleaching solution at the end of the latent period.

The bleaching process of our invention may be operated continuously. One method of continuous operation is to use a J-box of the type having a capacity such that the fabric remains in the J-box for from at least one and one-quarter hours to as long as two or more hours. The temperature of the solution and fabric in the J-box can be varied and the fabric may be removed from the J-box at such a rate that the time of the latent period may be substantially greater than one and one-quarter or one and one-half hours. When operating the bleaching process of this invention in a continuous manner, the same conditions and limitations apply as those found necessary and advantageous in batch bleaching operations.

Although our bleaching operation is particularly applicable to the bleaching of cottons of low grade for color it may also be practiced in the bleaching of white or unshaded cottons and results by a single bleaching operation in an improvement in the percent reflectance of such cottons and a degree of whiteness not obtainable by a conventional single bleaching operation.

This application is a continuation-in-part of our U. S. patent applications, Serial Numbers 199,468 and 199,469, filed December 6, 1950.

What is claimed is:

1. The method of bleaching cotton of low grade for color to a per cent reflectance of at least 88.5 Rd comprising the steps of: immersing the cotton in an inactive alkaline bleaching solution of a per compound for a minimum period of time of at least 1 1/4 to 1 1/2 hours, maintaining the temperature during a said period of time of at least 1 1/4 hours not substantially above 50° C., and during a said period of time of at least 1 1/2 hours not substantially above 55° C.; the amount of decomposition of the per compound while the cotton is immersed in the inactive alkaline bleaching solution for a period of time of not longer than about two hours being not greater than about twenty-six per cent; elevating the temperature of the bleaching solution to about 85° C., whereby the bleaching solution is activated; and maintaining the bleaching solution in an activated state until the per compound is substantially completely exhausted.

2. A method according to claim 1 in which the per compound is hydrogen peroxide.

3. A method according to claim 1 in which the per compound is sodium perborate.

4. The method of bleaching cotton of low grade for color; due to the presence of discolored matter within the lumina of the fibers, to a per cent reflectance of at least 88.5 Rd comprising the steps of: immersing the cotton in an inactive alkaline bleaching solution of a per compound for a minimum period of time of at least 1 1/4 to 1 1/2 hours, maintaining the temperature during a said period of time of at least 1 1/4 hours not substantially above 50° C., and during a said period of time of at least 1 1/2 hours not substantially above 55° C.; the amount of decomposition of the per compound while the cotton is immersed in the inactive alkaline bleaching solution for a period of time of not longer than about two hours being not greater than about twenty-six per cent; elevating the temperature of the bleaching solution to about 85° C., whereby the bleaching solution is activated; and maintaining the bleaching solution in an activated state until the per compound is substantially completely exhausted; and the discolored matter has been bleached.

5. The method of bleaching cotton of low grade for

color to a per cent reflectance of at least 88.5 Rd comprising the steps of: immersing the cotton in an inactive alkaline bleaching solution of a per compound for a minimum period of time of at least  $1\frac{1}{4}$  to  $1\frac{1}{2}$  hours, maintaining the temperature during a said period of time of at least  $1\frac{1}{4}$  hours within the range of from  $15^{\circ}$  C. to not substantially above  $50^{\circ}$  C., and maintaining the temperature during a said period of time of at least  $1\frac{1}{2}$  hours not substantially above  $55^{\circ}$  C.; the amount of decomposition of the per compound over the temperature range of  $15^{\circ}$  C. to about  $55^{\circ}$  C. while the cotton is immersed in the inactive alkaline bleaching solution for a period of time of not longer than about two hours being not greater than about twenty-six per cent; elevating the temperature of the bleaching solution to about  $85^{\circ}$  C., whereby the bleaching solution is activated; and maintaining the bleaching solution in an activated state until the per compound is substantially completely exhausted.

6. The method of bleaching cotton of low grade for color; due to the presence of discolored matter within the lumina of the fibers, to a per cent reflectance of at least 88.5 Rd comprising the steps of: immersing the cotton in an inactive alkaline bleaching solution of a per compound for a minimum period of time of at least  $1\frac{1}{4}$  to  $1\frac{1}{2}$  hours, maintaining the temperature during a said period of time of at least  $1\frac{1}{4}$  hours within the range of from  $15^{\circ}$  C. to not substantially above  $50^{\circ}$  C., and maintaining the temperature during a said period of time of at least  $1\frac{1}{2}$  hours not substantially above  $55^{\circ}$  C.; the amount of decomposition of the per compound over the temperature range of  $15^{\circ}$  C. to about  $55^{\circ}$  C. while the cotton is immersed in the inactive alkaline bleaching solution for a period of time of not longer than about two hours being not greater than about twenty-six per cent; elevating the temperature of the bleaching solution to about  $85^{\circ}$  C., whereby the bleaching solution is activated; and maintaining the bleaching solution in an activated state until the per compound is substantially completely exhausted and the discolored matter has been bleached.

7. The method according to claim 6 in which the per compound is hydrogen peroxide.

8. The method according to claim 6 in which the per compound is sodium perborate.

9. The method of bleaching cotton of low grade for color to a per cent reflectance of at least 88.5 Rd comprising the steps of: immersing the cotton in an inactive alkaline bleaching solution of a per compound selected from the class consisting of hydrogen peroxide, alkali metal peroxides, and inorganic per compounds which behave in aqueous solution as peroxides for a minimum period of time of at least  $1\frac{1}{4}$  to  $1\frac{1}{2}$  hours, maintaining the temperature during a said period of time of at least  $1\frac{1}{4}$  hours within the range of from  $15^{\circ}$  C. to not substantially above  $50^{\circ}$  C., and during a said period of time of at least  $1\frac{1}{2}$  hours maintaining the temperature not substantially above  $55^{\circ}$  C.; the amount of decomposition of the per compound over the temperature range of  $15^{\circ}$  C. to about  $55^{\circ}$  C. while the cotton is immersed in the inactive alkaline bleaching solution for a period of time of not longer than about two hours being not greater than about twenty-six per cent; elevating the temperature of the bleaching solution to about  $85^{\circ}$  C., whereby the bleaching solution is activated; and maintaining the bleaching solution in an activated state until the per compound is substantially completely exhausted and the discolored matter has been bleached.

10 of at least  $1\frac{1}{2}$  hours maintaining the temperature not substantially above  $55^{\circ}$  C.; the amount of decomposition of the per compound over the temperature range of  $15^{\circ}$  C. to about  $55^{\circ}$  C. while the cotton is immersed in the inactive alkaline bleaching solution for a period of time of not longer than about two hours being not greater than about twenty-six per cent; elevating the temperature of the bleaching solution to about  $85^{\circ}$  C., whereby the bleaching solution is activated; and maintaining the bleaching solution in an activated state until the per compound is substantially completely exhausted.

11. A method according to claim 9 in which the per compound is hydrogen peroxide.

12. A method according to claim 9 in which the per compound is sodium perborate.

13. The method of bleaching cotton of low grade for color; due to the presence of discolored matter within the lumina of the fibers, to a per cent reflectance of at least 88.5 Rd comprising the steps of: immersing the cotton in an inactive alkaline bleaching solution of a per compound selected from the class consisting of hydrogen peroxide, alkali metal peroxides, and inorganic per compounds which behave in aqueous solution as peroxides for a minimum period of time of at least  $1\frac{1}{4}$  to  $1\frac{1}{2}$  hours, 20 maintaining the temperature during a said period of time of at least  $1\frac{1}{4}$  hours within the range of from  $15^{\circ}$  C. to not substantially above  $50^{\circ}$  C., and during a said period of time of at least  $1\frac{1}{2}$  hours maintaining the temperature not substantially above  $55^{\circ}$  C.; the amount 25 of decomposition of the per compound over the temperature range of  $15^{\circ}$  C. to about  $55^{\circ}$  C. while the cotton is immersed in the inactive alkaline bleaching solution for a period of time of not longer than about two hours being not greater than about twenty-six per cent; elevating the temperature of the bleaching solution to about  $85^{\circ}$  C., whereby the bleaching solution is activated; and maintaining the bleaching solution in an activated state until the per compound is substantially completely exhausted and the discolored matter has been bleached.

14. A method according to claim 12 in which the per compound is hydrogen peroxide.

15. A method according to claim 12 in which the per compound is sodium perborate.

#### References Cited in the file of this patent

##### UNITED STATES PATENTS

|           |            |       |                |
|-----------|------------|-------|----------------|
| 1,278,389 | Schaidhauf | ----- | Sept. 10, 1918 |
| 2,220,682 | Kauffmann  | ----- | Nov. 5, 1940   |
| 2,530,244 | Jensen     | ----- | Nov. 14, 1950  |

##### FOREIGN PATENTS

|         |               |       |                |
|---------|---------------|-------|----------------|
| 637,140 | Great Britain | ----- | May 10, 1950   |
| 507,759 | Germany       | ----- | Sept. 22, 1930 |